

F. A. HAUGHTON.  
METHOD OF MAKING MANGANESE STEEL STAMP SHOES.  
APPLICATION FILED OCT. 19, 1911.  
1,033,800. Patented July 30, 1912.



Fig. 1.



Fig. 2.

Witnesses:  
P. M. Pittman  
F. E. Boyce.

Inventor  
Frank A. Haughton  
By his Attorney  
G. C. Reed

# UNITED STATES PATENT OFFICE.

FRANK A. HAUGHTON, OF HIGH BRIDGE, NEW JERSEY.

## METHOD OF MAKING MANGANESE-STEEL STAMP-SHOES.

1,033,800.

Specification of Letters Patent.

Patented July 30, 1912.

Application filed October 19, 1911. Serial No. 655,491.

To all whom it may concern:

Be it known that I, FRANK A. HAUGHTON, a subject of the King of Great Britain, residing at High Bridge, in the county of 5 Hunterdon and State of New Jersey, have invented certain new and useful Improvements in Methods of Making Manganese-Steel Stamp-Shoes, of which the following is a specification.

10 This invention relates to method of heat treating manganese steel stamp shoes, the object of the invention being to provide an improved stamp shoe which will embody all the good wearing qualities of manganese steel for crushing purposes and at the same time have the requisite degree of toughness at the point of juncture between the shank and the body thereof.

15 In the drawing accompanying and forming part of this specification, Figure 1 illustrates a stamp shoe made in the manner set forth; and Fig. 2 illustrates the manner in which the same is treated.

20 Similar characters of reference indicate 25 corresponding parts in the figures of the drawing.

Stamp shoes as usually made are so brittle that the shanks frequently break off, and this is the case especially when the shoes are 30 made of chilled cast iron. The heads of the stamp shoes are usually about nine inches in diameter, and owing to this large body of metal in the head of the shoe when made of manganese steel and treated in any of the 35 ways in which this steel is treated it has been found by actual experience that shrinkage cracks develop in the metal, extending over a considerable portion of the interior and at times extending to the outer 40 surface, so that the shoe is defective and incapable of performing the work for which it was designed. It is, however, essential that the metal adjacent to the point of juncture of the shoe body and its shank 45 be toughened, so that there will be no danger of the shank being broken from the body by the severe shocks which it receives in service, and I have discovered that by heating the shoe to the usual temperature to 50 which manganese steel is heated, as for instance about an orange heat, and immersing the shoe, shank downward, until the portion of the body immediately adjacent to the shank is submerged about an inch and a half 55 and allowed to remain in that state until the entire shoe is cold the shank and the portion

of the body adjacent thereto is toughened, while no shrinkage cracks develop in the body of the shoe. By this process I obtain a stamp shoe which embodies all the good 60 wearing qualities of manganese steel for crushing purposes, and at the same time obtain the requisite degree of toughness in the shank and in the body of the shoe adjoining such shank.

65 In manufacturing stamp shoes in the manner set forth, after the shoe is cast it is heated to the desired temperature and then immersed and supported by any suitable means, as 2, in a quenching bath, as 3, sufficiently to immerse the shank 4 and a portion 70 of the head 5 adjoining such shank, and there allowed to remain until the entire shoe is cold, whereupon it is removed. By this process it has been found, as hereinbefore 75 stated, that the shank and that portion of the body adjacent thereto is thoroughly toughened, and that no shrinkage cracks develop in the body of the shoe, while the remaining portion of the body is sufficiently 80 tough to fulfil all the requirements of a stamp shoe.

I claim as my invention:

1. The method of heat treating manganese steel stamp shoes comprising a body 85 and shank which consists in heating and then immersing a part of the shoe in a quenching bath, with the shank thereof downward, to a point beyond the juncture point of the body and the shank and allowing 90 the same to cool.

2. The method of heat treating manganese steel stamp shoes comprising a body and shank which consists in heating and then immersing a part of the shoe in a 95 quenching bath, with the shank thereof downward, to a point beyond the juncture point of the body and the shank and allowing the same while so immersed to cool.

3. The method of heat treating cast manganese steel stamp shoes, comprising a body and a shank, which consists in heating it up to a substantially orange heat, and then immersing it in a quenching bath, with the shank thereof downward, to a point beyond 105 the juncture point of the shank and the body so that the entire shank and a portion of the body will be immersed in such bath and while so immersed allowing it to become cool.

4. The method of heat-treating manganese steel stamp shoes comprising a body

110

and shank, which consists in heating the same and then rapidly cooling that part of the shoe comprising the shank and body to a point slightly beyond the juncture point of such shank and body.

5. The method of heat-treating manganese steel stamp shoes comprising a body and shank, which consists in heating the same and then immersing in a quenching bath the shank and a part of the body to a

point beyond the juncture point of such body and shank and allowing the same to cool.

Signed at High Bridge, N. J., this 13th day of October, 1911.

FRANK A. HAUGHTON.

Witnesses:

E. B. COSS,  
H. W. WYCKOFF.

Copies of this patent may be obtained for five cents each, by addressing the "Commissioner of Patents, Washington, D. C."